

Aug. 3, 1943.

G. F. NADEAU ET AL

2,326,056

ANTIHALATION FILM

Original Filed March 4, 1941

Fig. 1



Fig. 2



Gale F. Nadeau  
Alfred D. Slack  
INVENTORS

BY *Newton M. Perrin*  
*R. Frank Smith*  
ATTORNEYS

Patented Aug. 3, 1943

2,326,056

# UNITED STATES PATENT OFFICE

2,326,056

## ANTIHALATION FILM

Gale F. Nadeau and Alfred D. Slack, Rochester, N. Y., assignors to Eastman Kodak Company, Rochester, N. Y., a corporation of New Jersey

Original application March 4, 1941, Serial No. 381,695. Divided and this application November 1, 1941, Serial No. 417,530

6 Claims. (Cl. 95—8)

This invention relates to a photographic film and more particularly to a film provided with antihalation layers.

This application is a division of Nadeau and Slack U. S. Patent 2,311,073, granted February 16, 1943.

Coatings on the backs of films containing a dye or a superficial dye layer removable in photographic processing solutions are well known for antihalation purposes. Less well known are antihalation layers which are designed to be nonremovable. The disadvantages of the removable types of coatings are the tendency of some coatings to deposit sludge in processing solutions, the tacky nature of some coatings, the known thermoplastic qualities of other coatings which are in general undesirable, and furthermore, in the case of certain resinous coatings their tendency to form insoluble products with the antihalation dye. Non-removable antihalation layers have been designed to avoid these difficulties and to prevent the penetration of the dye into and the consequent staining of the support. The success of this practice depends upon the selection of a material, for the dye carrier, which is sufficiently permeable to processing solutions, yet not soluble, that the dye giving antihalation protection may be completely discharged when desired.

The object of the present invention is to provide a photographic film with a carrier for an antihalation dye, said carrier being permeable to, but not soluble in, photographic processing solutions. Other objects appear hereinafter.

We have found that a cellulose organic acid dicarboxylic acid ester containing substantially 4-8 acyl groups per  $C_{24}$  cellulose unit, of which not more than one is a dicarboxylic acid acyl group and the remainder are aliphatic monobasic acid acyl groups of less than five carbon atoms, accomplishes our objects when used as an antihalation layer in conjunction with a dye.

The general method we employ is to coat a photographic support with an emulsion, joining said emulsion to the support by means of suitable subbing layers. We then coat a water-permeable cellulose ester layer and a dye layer onto the other side of the support. We may vary this procedure by applying the antihalation layer between the light sensitive emulsion layer and the support. The antihalation layer may also be coated before the emulsion layer.

Fig. 1 represents the general method of applying an antihalation layer and a dye to the back of a film support provided on the front side with

a light sensitive layer adhesively joined to the support by means of a subbing layer.

Fig. 2 represents a multi-layer color film provided, on one side of a subbed cellulose acetate propionate support, with emulsion layers sensitive to red, green and blue light, and on the opposite side, a cellulose acetate phthalate antihalation layer containing a dye.

According to the preferred method of our invention we used an antihalation layer consisting of a cellulose organic acid dicarboxylic acid ester containing substantially 4-8 acyl groups, but not more than one dicarboxylic acid acyl group per  $C_{24}$  cellulose unit, in intimate contact with a dye layer. We have particularly chosen cellulose esters of this range of acyl content because of their characteristic permeability to water. For instance, cellulose acetate phthalates of this class containing less than 4 acyl groups or more than one phthalyl group per  $C_{24}$  cellulose unit are too soluble in photographic processing solutions to be of use in the manner of our invention. Likewise, those esters containing more than 8 acyl groups are too impermeable to be used in our invention. It is obvious that we contemplate the use of other cellulose organic acid dicarboxylic acid esters, such as cellulose acetate propionate phthalate, cellulose acetate butyrate phthalate, cellulose acetate succinate, etc., the acyl content of which is of the order described.

In designating the cellulose esters of our invention in terms of acyl groups, we use the expression "substantially." This is due to the fact that in analyzing our esters we find that those esters which are useful fall within the range approximated by those esters having 4-8 acyl groups  $C_{24}$  cellulose unit. Thus, cellulose acetate phthalate containing more than about 14 per cent phthalyl, in addition to about 7 acyl groups per  $C_{24}$  unit is too permeable to photographic developing solutions to be of use in our invention and this phthalyl content corresponds to about 1 phthalyl group per  $C_{24}$  unit of cellulose. We use a  $C_{24}$  unit as the basic cellulose unit in order to avoid expressing the dicarboxylic acid acyl content of an ester in fractional terms in respect to the aliphatic monobasic acid acyl content.

Several types of supports may be provided with the antihalation layer of our invention. Cellulose esters such as cellulose acetate or cellulose nitrate, or mixed esters of cellulose, such as cellulose acetate propionate and cellulose acetate butyrate, and opaque supports such as paper, may all be so provided with antihalation

layers. Dyes which are removable in ordinary photographic processing solutions are applicable for use in conjunction with the cellulose ester antihalation layers we describe. These dyes are commonly known as fugitive dyes. The dye may be applied to the antihalation carrier layer by dispersing it in an organic solvent such as a mixture of methanol and water; or ethanol, water and methyl Cellosolve in suitable proportions.

We will now describe our invention with particular reference to the accompanying drawing.

As shown in Fig. 1 of the accompanying drawing a cellulose ester support 10 is provided with a subbing layer 12 which may be gelatin or other suitable material, and over this is coated the emulsion layer 13 which may consist of a silver halide and colloid, such as gelatin, a cellulose or resinous material. On the opposite side of the support is coated the antihalation layer 11 of our invention containing a dye in the outer stratum.

Fig. 2 shows a multilayer color film wherein a cellulose acetate propionate support 10 is provided with the red, green and blue light sensitive emulsion layers 14, 15, and 16 respectively, adhesively joined to the support by means of a subbing layer 12. On the opposite side of the support is an antihalation layer 11 consisting of a cellulose acetate phthalate, 14-28% acetyl and 0-14% phthalyl, containing a dye in the outer stratum.

The following example illustrates one method of producing a film according to our invention, said example being intended to merely illustrate our invention and is not to be taken as limiting the scope of said invention.

#### Example

A film base of cellulose acetate propionate containing 16% propionyl and 29% acetyl is coated with a 3% solution of cellulose acetate phthalate, acetyl content 25% and phthalyl 13%, in a mixture of 45 parts acetone and 55 parts of methanol. Over this layer is applied a fugitive type of dye such as Acid Blue 2R or a dye of Color Index No. 702, 704, 705, or 707. The solvent mixture for the dye may vary over a fairly wide range, although a mixture of 90 parts of methanol and 10 parts of water is generally satisfactory. On the other side of the support, now provided with an antihalation layer, is coated from solvent solution, a subbing layer consisting of a resin or a mixture of a resin and a cellulose ester followed by a gelatin layer and a light sensitive emulsion layer. Resins containing subbing layers have been more fully described in a prior Patent U. S. 2,133,110, and others. A subbing solution, containing gelatin and which is suitable for coating a gelatin layer over a resin containing layer is also described therein. The film may be provided with differentially light-sensitive emulsion layers which may be sensitized in the natural order as shown in Fig. 2 of the drawing, or sensitized in the natural order and colored complementary to the sensitivity as desired. A filter dye may be incorporated in one of the layers such as the blue sensitive layer in order to screen the lower layers from radiations which they are not intended to record. Also, there may be interposed between the emulsion layers a layer designed to receive a sound record or this record may be printed in one of the emulsion layers. It is obvious that we may reverse or vary the order of deposition of the

layers on the support as in an alternative method we coat the emulsion layers on the support before the antihalation and dye layers.

The photographic elements described are used in any of the well-known processes designed to record an image in black-and-white or color. After exposure of the materials to an image the elements are usually developed to a negative and during this development or in a subsequent fixing treatment the cellulose ester antihalation layer becomes sufficiently swollen to allow the penetration of the constituent removing the antihalation dye, but the cellulose ester of the antihalation layer is not dissolved.

While we have described the use of permeable cellulose esters, in antihalation layers, and this is the preferred embodiment of our invention, it is evident that any process requiring a water permeable, but not soluble layer, with or without a dye, may be served by the materials of our invention. Such processes are those of the photographic type which use sensitive films containing light filtering layers, the dye of which is to be removed at some stage in the processing treatment.

The materials and examples of the present specification are illustrative only and it is to be understood that numerous methods and ingredients may be used within the scope of the present description, and that the scope of our invention is to be taken as limited only by the scope of the appended claims.

What we claim is:

1. A photographic element free from halation which comprises a support provided with a light sensitive emulsion layer, and an antihalation layer of a water-permeable cellulose ester containing substantially 4 to 8 acyl groups per  $C_{24}$  cellulose unit, of which one is a dicarboxylic acid acyl group and the remainder are aliphatic monobasic acid acyl groups of less than five carbon atoms, said layer carrying a light-absorbing dye.

2. A photographic element free from halation which comprises a support provided with a light sensitive emulsion layer, and an antihalation layer of a water-permeable cellulose ester containing substantially 4 to 8 acyl groups per  $C_{24}$  cellulose unit, of which one is a phthalyl group and the remainder are aliphatic monobasic acyl groups of less than five carbon atoms, said layer carrying a light-absorbing dye.

3. A photographic element free from halation which comprises a support provided with a light sensitive emulsion layer, and an antihalation layer of a water-permeable cellulose ester containing substantially 4 to 8 acyl groups per  $C_{24}$  cellulose unit, of which one is a phthalyl group and the remainder are acetyl groups, said layer carrying a light-absorbing dye.

4. A photographic element free from halation which comprises a support provided with a light sensitive emulsion layer, and an antihalation layer of a water-permeable cellulose ester containing, per  $C_{24}$  cellulose unit, substantially one phthalyl group and seven acetyl groups, said layer carrying a light-absorbing dye.

5. A photographic element free from halation which comprises a cellulose acetate propionate support provided with a light sensitive emulsion layer, and an antihalation layer of a water-permeable cellulose ester containing, per  $C_{24}$  cellulose unit, substantially one phthalyl group and seven acetyl groups, said layer carrying a light-absorbing dye.

6. A photographic element free from halation which comprises a support provided with a light sensitive emulsion layer, and an antihalation layer of a water-permeable cellulose aliphatic monobasic organic acid-dicarboxylic acid, ester containing substantially 4 to 8 aliphatic monobasic organic acid acyl and dicarboxylic acid acyl

groups per C<sub>24</sub> cellulose unit, of which not more than one is a dicarboxylic acid acyl group and the remainder are aliphatic monobasic acid acyl groups of less than five carbon atoms, said layer carrying a light-absorbing dye.

GALE F. NADEAU.  
ALFRED D. SLACK.